

March 19, 1935.

W. SCHNEIDER ET AL

1,994,876

PHOTOGRAPHIC FILM FREE FROM HALATION

Filed Feb. 18, 1932



By

Inventors:  
Wilhelm Schneider,  
Konrad Hobbel,  
Philip S. Hopkins,  
Attorney.

## UNITED STATES PATENT OFFICE

1,994,876

PHOTOGRAPHIC FILM FREE FROM  
HALATION

Wilhelm Schneider, Dessau in Anhalt, and Konrad Hebbel, Wolfen, near Bitterfeld, Germany, assignors to Agfa Ansco Corporation, Binghamton, N. Y., a corporation of New York

Application February 18, 1932, Serial No. 593,918  
In Germany November 5, 1929

## 6 Claims. (Cl. 95—9)

Our present invention relates to new photographic films and more particularly to films free from halation. It is a continuation in part of our copending application Ser. No. 491,619, filed October 27, 1930.

The object of our present invention is to provide a photographic film free from halation having applied to its back side an intermediate layer swellable in water or in aqueous solutions, said 10 intermediate layer bearing the proper anti-halation layer. Further objects will be seen from the detailed specification following hereafter.

We have found that the support of a film carrying on one of its faces a light sensitive emulsion layer is protected from being undesirably colored when providing an anti-halation on its back side by applying the said anti-halation layer not directly to the support, but to an intermediate layer of any material which swells in water or in aqueous 15 solutions, for instance, the photographic baths. Such swellable materials adapted for the preparation of an intermediate layer are gelatin, albuminous substances or casein rendered insoluble in water by a treatment with hardening agents 20 but still remaining swellable, cellulose ethers swellable in water or the like. The thickness of the intermediate layer may vary within wide 25 limits.

For example we may provide on the support a 30 gelatin layer of about  $1 \mu$  thickness made in the same manner as the sub-coating for a light sensitive emulsion layer, or we may use a thicker intermediate layer up to about  $30 \mu$  by applying to the sub-coating a usual non-curling layer. These 35 layers are applied to the support according to known methods.

The anti-halation layer proper, comprising one 40 dye or a mixture of several dyes with or without the use of a binding agent, is applied to the intermediate layer. The anti-halation dyes which we prefer are those soluble in alkaline liquids and capable of forming a coherent smooth layer when cast from which no particles split off. Such dyes 45 are for instance, the fuchsones and the fuchson imides.

If desired, for rendering the photographic material entirely free from halation, when using a mixture of dyes one or more of the dyes which do, however, not tend to permanently color the film 50 may be incorporated in the intermediate layer. Appropriated for this purpose are, for instance, methyl blue (see Schultz, Farbstofftabellen, 5<sup>th</sup> edition No. 537) giving a blue color, alkali blue (see Schultz, Farbstofftabellen, 5<sup>th</sup> edition No. 536) likewise giving a blue color, acid fuchsin (see

Schultz Farbstofftabellen, 5<sup>th</sup> edition No. 524) giving a bluish red color, 3,4-dimethoxy-styryl-quinoline-dimethylsulfate of the formula



5 giving a yellow color and 4-dimethylamino-10 styryl-quinoline-dimethylsulfate giving a red color. The color of the dyes incorporated in the intermediate layer is preferably chosen in such a manner as to cover the gaps of absorption of the proper anti-halation layer as far as the light sensitive emulsion is sensitive to the waves of these 15 gaps.

The following examples illustrate our invention:—

Example 1.—To a nitrocellulose film as used for photographic materials, there is applied in known manner a very thin layer which may be made from a solution of

|                     |          |    |
|---------------------|----------|----|
| Gelatin             | 60 grams | 25 |
| Glycerol            | 150 cc.  |    |
| Glacial acetic acid | 20 cc.   |    |
| Water               | 150 cc.  |    |
| Methanol            | 2000 cc. |    |
| Acetone             | 7000 cc. | 30 |

In order to obtain a film entirely free from halation, this layer may after drying be colored by bathing the film in an aqueous solution of a dye which does not tend to color the support, for instance, in an aqueous solution of methyl blue. When the intermediate layer is dry, an anti-halation layer of  $0.5$  to  $1 \mu$  thickness, obtained from a solution containing 500 grams of aurine (Schultz, Farbstofftabellen, 5<sup>th</sup> edition, No. 555) and 10 liters of alcohol is applied thereon. The anti-halation layer thus prepared has a smooth surface and can be removed within a short time in the usual photographic developers.

Example 2.—A support of cellulose acetate is in known manner provided with a sub-coating. To the support thus prepared there is applied a non-curling layer, made from a solution of 1 kilo of gelatin in 9 liters of water to which 100 cc of a solution of chrome alum have been added. This 45 solution in which there are dissolved 2-10 grams of methyl blue per kilo is applied at a temperature of about  $35^{\circ}$  C. in a manner as to obtain a uniform gelatin layer of the desired thickness of say 50 20 to 25  $\mu$ . After the intermediate non-curling 55

layer has dried an anti-halation layer of 0.5 to 1  $\mu$  thickness, obtained from a solution containing 500 grams of aurine and 10 liters of alcohol is applied thereon.

5. *Example 3.*—The conditions are the same as in Example 2 with the difference that the solution for preparing the intermediate layer contains 2 to 10 grams of acid fuchsin per kilo and that the proper anti-halation layer is made from a solution of 1 kilo of benzaurine in 10 liters of propanol.

10. *Example 4.*—The conditions are the same as in Example 2 with the difference that the solution for preparing the intermediate layer contains 1 to 5 grams of 4-dimethylamino-styryl-quinoline-dimethylsulfate per kilo and that the proper anti-halation layer is made from a solution of 750 grams of aurine-tri-carboxylic-acid in 10 liters of isobutanol.

15. *Example 5.*—The conditions are the same as in Example 2 with the difference that the solution for preparing the intermediate layer contains 1 to 5 grams of 3,4-dimethoxy-styryl-quinoline-dimethylsulfate and that the proper anti-halation layer is made from a solution of 250 grams of oxytolylaminofuchsoncarboxylic acid in 10 liters of propanol.

20. *Example 6.*—The conditions are the same as in Example 5 with the difference the proper anti-halation layer is made from a solution of 1 kilo of fuchsin-tri-carboxylic-acid in 10 liters of alcohol.

25. In the accompanying drawing a photographic film is shown in cross section and on an enlarged scale, illustrating the peculiar features of our invention.

30. In this drawing *a* is the photographic emulsion applied to the emulsion carrier, *b*, consisting, for instance, of nitrocellulose or another cellulose derivative, *c* is the intermediate layer swellable in water or in the photographic baths. *d* is the anti-halation layer.

35. Our present invention is not limited to the foregoing examples nor to the specific details given therein. Intermediate layers made from other substances than those mentioned are possible comprising one or more strata. These layers may be dyed with dyestuffs having no affinity to the film support, or they may be used undyed according to the purpose in question. These dyes

40. must furthermore have the property of being removable or decolorized in the photographic baths preferably in the alkaline developer in such a manner that the intermediate layer will remain colorless regardless of any further treatment. The proper anti-halation layer may be made from any dye that will form a coherent layer from which particles do not split off and which layer is soluble in the photographic baths. The thickness

45. of the intermediate layer and of the anti-halation layer may vary within wide limits and is to be chosen according to the desired purpose. A few simple experiments will be sufficient to determine in each particular case the best conditions and the most suitable amount of dyestuff to be used.

50. Other embodiments than those given in the ex-

amples are possible and we contemplate as included within our invention all such modifications as fall within the scope of the appended claims.

5. What we claim is:—

1. A photographic film free from halation and comprising an emulsion carrier consisting of cellulosic material coated on one side with a photographic emulsion and on the other side with an intermediate layer swellable in aqueous solutions or in water, and on the outer surface of said intermediate layer an anti-halation dye soluble in feebly alkaline baths but insoluble in water.

10. 2. A photographic film free from halation and comprising an emulsion carrier consisting of cellulosic material coated on one side with a photographic emulsion and on the other side with an intermediate layer consisting of a material swellable in aqueous solutions or in water and on the outer surface of said intermediate layer an anti-halation layer soluble in feebly alkaline baths but insoluble in water.

15. 3. A photographic film free from halation and comprising an emulsion carrier consisting of cellulosic material coated on one side with a photographic emulsion and on the other side with an intermediate layer consisting of a material swellable in aqueous solutions or in water and in which is incorporated an anti-halation dye having no affinity for dyeing permanently the cellulosic material, and on the outer surface of said intermediate layer an anti-halation layer soluble in feebly alkaline baths but insoluble in water.

20. 4. A photographic film free from halation and comprising an emulsion carrier consisting of a cellulosic material coated on one side with a photographic emulsion and on the other side with an intermediate layer consisting of a material swellable in aqueous solutions or in water and which is dyed with methyl blue, and on the outer surface of the intermediate layer an anti-halation layer comprising aurine.

25. 5. A photographic film free from halation and comprising an emulsion carrier consisting of a cellulosic material coated on one side with a photographic emulsion and on the other side with an intermediate layer consisting of a material swellable in aqueous solutions or in water and which is dyed with 4-dimethylamino-styryl-quinoline-dimethyl-sulfate, and on the outer surface of the intermediate layer an anti-halation layer comprising aurine-tri-carboxylic-acid.

30. 6. A photographic film free from halation and comprising an emulsion carrier consisting of a cellulosic material coated on one side with a photographic emulsion and on the other side with an intermediate layer consisting of a material swellable in aqueous solutions or in water and which is dyed with 3,4-dimethoxy-styryl-quinoline-dimethylsulfate, and on the outer surface of the intermediate layer an anti-halation layer comprising oxytolylaminofuchsoncarboxylic acid.

35. WILHELM SCHNEIDER.  
KONRAD HEBBEL.